

No. 715,584.

Patented Dec. 9, 1902.

W. KENT.

WELDED CAST METAL PROCESS.

(Application filed Apr. 15, 1901.)

(No Model.)

Fig. I



Fig. II



Fig. III



Fig. IV



Fig. V



Inventor,

William Kent

Witness:

Banko Q. Rose  
Chas H. Urban

By his Attorney,

J. W. H. Clay

# UNITED STATES PATENT OFFICE.

WILLIAM KENT, OF COVINGTON, KENTUCKY.

## WELDED CAST-METAL PROCESS.

SPECIFICATION forming part of Letters Patent No. 715,584, dated December 9, 1902.

Application filed April 15, 1901. Serial No. 55,810. (No specimens.)

*To all whom it may concern:*

Be it known that I, WILLIAM KENT, a citizen of the United States, residing at Covington, in the State of Kentucky, have invented 5 a certain new and useful Welded Cast-Metal Process, of which the following is a specification.

My invention relates to the iron-working art, and has for its object, primarily, to 10 strengthen cast iron or steel by intimately mixing with it a quantity of wrought iron or steel. It also consists in a composite material composed of high-carbon iron or steel and low-carbon iron or steel welded together. in 15 the act of casting and more intimately mixed by rolling.

In the use of iron there are often cases 20 where the rigidity and hardness of cast-iron or steel is needed without the tensile strength of wrought iron or steel, and yet because the cast metal is brittle it cannot be used for fear of breaking under accidental jars and sudden strains. On the other hand, to use enough of the wrought metal to obtain 25 the desired rigidity involves too great expense and requires too great a bulk of metal. The essential difference between the hard cast or high-carbon metal and the soft wrought or low-carbon metal is not so much 30 chemical as structural. The former is crystalline, having no fiber. The latter is laminated in structure with a long fiber or "grain" in the mass. The best puddled iron, even when it has more carbon than certain cast- 35 steels, is yet tougher and more malleable than the latter. It is therefore plain that the toughness is due to the internal structure, the fibrous weaving that is attained by the mechanical operation of puddling and roll- 40 ing. The object of my invention then is to produce this kind of structure in a composite metal by interspersing filaments of wrought iron or steel in a mass of cast iron or steel in the act of casting and weave them in the mass 45 by rolling rather than by mechanically mixing by stirring in the puddle while the metal is liquid.

Certain irons, like "Bessemer cast," for example, while they may be rolled when hot become brittle when cold. I prefer to use this 50 class of cast metal, and I give it tensile strength and overcome its brittleness by in-

corporating in its mass various fibers of wrought metal welded in with it.

In the accompanying drawings, Figure I 55 illustrates an arrangement of bars in the mold. Fig. II shows the use of chains for the purpose. Fig. III is a section of the ingot. Fig. IV indicates the effect of rolling; and Fig. V is a view of an armor-plate with a section showing irregular portions of wrought metal, as from the use of chains in casting.

The cold wrought iron or steel is arranged in an ingot-mold *c*, so that the size of the pieces *b* varies inversely with the distance of 65 the piece from zone of greatest heat—that is, the center of the mold. Then I pour in the molten high-carbon iron or steel *a* at a sufficient temperature to fuse the wrought metal, when the heat imparted to it brings it to the 70 welding state and the two become thoroughly welded together. The oxid in the fusing and in the subsequent rolling is displaced and allows full welding while itself adding strength to the composite metal by toughening the 75 grain. The ingot may then be rolled into the desired form, and the metal will have in a large measure the qualities of both cast and wrought metal, these qualities being improved by rolling and working, which more 80 intimately incorporates the two metals and further intermixes the oxid slag.

By properly proportioning the amount of wrought metal *b* and properly locating it so that the largest pieces get the greatest or 85 longest exposure to the heat of the molten metal *a* a thorough welding takes place. I may use wires or bars of new iron, or old chains, or loose scraps or cuttings, or a specially-designed structure to evenly distribute the 90 metal.

After the casting step, by which the wrought metal is distributed in the mass of cast metal in various small masses, so arranged as to facilitate the welding and the subsequent distortion and compression due to rolling, (placing more wrought metal in the interior for this purpose,) the masses of wrought metal and the oxid must be interwoven in the mass to get the desired internal structure. The 100 ingot is then heated in the "pickling" or cementation furnace, softening without oxidation to fit it for compressing, and is then rolled and worked up thoroughly, during which step

of the process these small masses of wrought metal and oxid are entirely broken down, displaced, and interwoven throughout the mass of cast metal, this distribution being 5 facilitated by the fact that the cast metal is harder and the wrought metal crushes easily. The result is that the cast metal itself is given a striated or fibrous structure rather than the crystalline, and there are intermixed and 10 woven all through it the filaments of wrought metal irregularly distributed in somewhat the manner attained by puddling, above referred to. It is this internal weaving of the fibers which gives the desired quality and which is 15 the object of this process.

Probably the properties and the function of my composite metal may best be illustrated by referring to its adaption to use in armor-plate.

20 In the former making of armor-plate malleable metal was used, and in that case the penetration of the projectile did not destroy the plate or do any more injury than results from the penetration of wooden sides. It was 25 afterward sought to prevent penetration by hardening the metal; but in this case even the slightest penetration of the projectile causes the entire disruption of the plate, because of its brittleness. The first attempt to 30 overcome this difficulty was made by Warden in 1862, when he cast a plate about a central framework of wrought-iron. In case of fracture this had an action similar to the action of hair in plasterers' mortar—that is, it did 35 not serve to prevent a fracture in any degree, (the two metals not being welded together,) but merely served to prevent the pieces from entirely dropping apart after they were fractured. Now my invention is de- 40 signed, first, to use for the main bulk of the metal a cheaper grade of iron or steel; sec- ond, to form a hard resisting outer surface to prevent as much as possible any penetration of the projectile, and, third, to provide the 45 metal with a laminated fibrous structure, giving it tensile strength, so that it will with- stand a very heavy blow without producing a fracture—that is, a plate will have the ad- vantage of hardness and rigidity, due to high 50 carbon or cast iron or steel, and yet avoid their objectionable brittleness, so that less weight or thickness need be used to obtain the same resistance to breaking. The plate will hold together even when entirely pene- 55 trated, and at the same time the resistance to penetration that was obtained in the cast-steel plate is preserved.

The process when applied to the manufac- ture of shafting, rails, and structural iron, 60 particularly for columns, is even more val- uable, for there are many places where cast

columns may not be used because of the dan- ger that a sudden jar will rupture them, while, on the other hand, malleable columns may not be used because they have not sufficient ri- 65 gidity.

Of course this composite metal may be used in directly casting articles in their final form—as, for example, large shafts and columns; but the filaments of wrought metal must be 70 distributed throughout the whole mass, and the process is distinguished from those in which the wrought metal is merely embedded in the cast metal.

Having thus described my invention and its 75 use, I desire to secure by Letters Patent of the United States the following, and I claim—

1. The process of making composite crys- talline and fibrous metal by arranging in an 80 ingot-mold a series of filaments or pieces of wrought-iron, then pouring in and around the same molten "cast" or high-carbon iron heat- ed to a temperature just sufficient to weld the two metals together, and afterward rolling and working the ingot to further incorporate 85 and distribute the wrought metal through the cast metal, and break down the form of the wrought pieces whereby the mass retains the hardness of cast-iron while possessing a woven fibrous internal structure of thoroughly in- 90 corporated laminae of oxid and soft iron.

2. The process of making composite crys- talline and fibrous metal by first placing in a 95 mold various masses of wrought-iron arranged in sizes varying with the distance from the side walls of the mold, then pouring in and around the same molten "cast" or high-car- bon iron at a temperature just sufficient to weld the two metals where in contact, and afterward rolling and working the whole mass 100 to break up the form of the wrought pieces and thoroughly interweave and distribute the wrought metal, giving the mass a partly fibrous and partly crystalline internal struc- ture.

3. The armor-plate composed of compound 105 cast and wrought iron or steel, the wrought metal being in the form of irregular filaments varying in size approximately with their dis- tance from the outside surface, welded and 110 woven in the mass of cast metal, both metals being crushed and distorted out of their orig- inal cast position and form by subsequent roll- ing, so that the cast metal is rendered fibrous rather than crystalline, as set forth.

In testimony whereof I have hereunto signed my name in the presence of the two 115 subscribing witnesses.

WILLIAM KENT.

Witnesses:

BERTHA O. ROSS,  
CHAS. H. URBAN.